

## 1

3,674,471  
ALLOY

A. David Joseph, New Canaan, Conn., assignor to  
Eutectic Corporation, Flushing, N.Y.  
No Drawing. Filed Apr. 9, 1970, Ser. No. 27,138  
Int. Cl. C22c 9/02, 9/06  
U.S. Cl. 75—153

1 Claim

## ABSTRACT OF THE DISCLOSURE

A copper base alloy with silver, phosphorus and tin additions that has self wetting properties that permit deposition by welding upon aluminum bronze and manganese bronze type base metals.

Heretofore it has been known in the art that it is difficult to weld upon aluminum bronze and manganese bronze type base metals. The surface oxides on the aluminum and manganese bronzes are difficult to remove and their presence creates difficulties when weld depositing an alloy weld deposit on these metals. These difficulties include unsatisfactory wetting, bond line porosity and surface impurities.

It is the general object of the present invention to avoid the difficulties of the prior art practices by providing an alloy with good wetting properties for weld deposition on aluminum and manganese bronzes.

Another object of the present invention is to provide a machineable alloy capable of being weld deposited by flame spraying.

Yet another object of this invention is to provide an alloy for weld deposition on aluminum and manganese bronze base metals without melting the base metal.

Extensive experimental work with copper base alloys led to the discovery that a copper base alloy with phosphorous, silver and tin additions generated exceptional surface wetting properties. In continued experimentation modifications of these alloys were weld deposited by various processes including the flame spraying of a powder (finer than 25 mesh size) version of these alloys, on base metals of the aluminum bronze class and the manganese bronze class with exceptionally good results. The alloys displayed exceptional surface wetting properties and a melting point that permitted deposition on aluminum and manganese bronze base metals without any melting of the base metals. Further experimentation led to the development of these alloys with the foregoing properties and in addition with good machineability.

The alloys of the present invention comprise the following alloy composition in the weighted percentages indicated:

| Element: | Weight percent |         |
|----------|----------------|---------|
|          | Range          | Example |
| Ag       | 2 to 12        | 9       |
| P        | 3 to 7         | 6       |
| Sn       | 1 to 5         | 5       |
| Ni       | 0 to 2         | 1       |
| Cr       | 0 to 1         | 1       |
| Si       | 0 to .5        | 0.2     |
| Fe       | 0 to .5        |         |
| B        | 0 to .4        | .1      |
| C        | 0 to trace     |         |
| Cu       | Balance        | Balance |

## 2

The alloy can be provided as a cast rod or in powder form. The powder can be manufactured by any of the well known processes such as by atomization.

In addition the alloy can be provided upon weld deposition from a heterogeneous powder mixture of several powder alloys finer than 25 mesh size. An example of a heterogeneous powder mixture is the following:

| Element                                         | Weight percent |
|-------------------------------------------------|----------------|
| 0 to 3 by weight of the following alloy powder: |                |
| C                                               | .65            |
| Cr                                              | 16.0           |
| Si                                              | 4.0            |
| Fe                                              | 3.5            |
| B                                               | 3.2            |
| Ni                                              | Bal.           |

mixed with 8 to 12% by weight of the following alloy powder:

|    |    |
|----|----|
| Cu | 72 |
| Ag | 28 |

mixed with 25 to 35% by weight of the following alloy powder:

|    |      |
|----|------|
| Sn | 8    |
| P  | 0.3  |
| Cu | Bal. |

mixed with 48 to 67% by weight of the following alloy powder:

|    |      |
|----|------|
| P  | 7.5  |
| Cu | Bal. |

It will be understood by those skilled in the art that the foregoing example is offered only as an example and that a good number of heterogeneous powder combinations can practice the spirit of the invention where a number of alloy powders in a heterogeneous combination can weld deposit the invention alloy.

It will now be understood by those skilled in the art that the objects of the invention have been achieved by providing a copper base alloy with exceptional wetting properties.

I claim:

1. An alloy consisting essentially of the following constituents in the weight percentages indicated:

| Constituent: | Weight percent |
|--------------|----------------|
| Ag           | 9              |
| P            | 6              |
| Sn           | 5              |
| Ni           | 1              |
| Cr           | 1              |
| Si           | 0.2            |
| B            | 0.1            |
| Cu           | Balance        |

## References Cited

## UNITED STATES PATENTS

|           |         |              |        |
|-----------|---------|--------------|--------|
| 1,921,416 | 8/1933  | Leach        | 75—154 |
| 1,988,422 | 1/1935  | Miller       | 75—154 |
| 2,390,775 | 12/1945 | Christ       | 75—154 |
| 3,392,017 | 7/1968  | Quaas et al. | 75—154 |

CHARLES N. LOVELL, Primary Examiner

65 U.S. Cl. X.R.

75—154, 159, 160

UNITED STATES PATENT OFFICE  
CERTIFICATE OF CORRECTION

Patent No. 3,674,471 Dated July 4, 1972

Inventor(s) A. David Joseph

It is certified that error appears in the above-identified patent and that said Letters Patent are hereby corrected as shown below:

Column 2, Line 9, after "3" add a percent sign --%--.

Column 2, Line 19, delete "Cu" and add --Ag--.

Column 2, Line 20, delete "Ag" and add --Cu--.

Signed and sealed this 24th day of October 1972.

(SEAL)

Attest:

EDWARD M.FLETCHER, JR.  
Attesting Officer

ROBERT GOTTSCHALK  
Commissioner of Patents